

## UNITED STATES PATENT OFFICE

2,019,185

ARTIFICIAL FIBER AND PROCESS OF  
PRODUCING SAMERudolph H. Kagi, Grantwood, N. J., assignor to  
Heberlein Patent Corporation, New York, N. Y.,  
a corporation of New YorkNo Drawing. Application February 27, 1933,  
Serial No. 658,838. In Germany March 10,  
1932

13 Claims. (Cl. 117—53)

This invention relates to the improvement of artificial fibers, especially artificial silk. The known products of artificial silk possess a greater brittleness than natural fibers. Through various finishing treatments this characteristic can be eliminated somewhat, but insufficiently. It has already been proposed to increase the elasticity of artificial fibers by chemical action, but up to the present time no real success has been attained

10 in this direction.

The principal object of the present invention accordingly is to produce an artificial silk possessing novel characteristics and especially one in which the objectionable characteristic mentioned 15 is substantially reduced or eliminated. Another object is to provide a simple and efficient process for producing this material.

The invention comprises the novel products as well as the novel processes and steps of processes 20 according to which such products are manufactured, the specific embodiments of which are described hereinafter by way of example and in accordance with which I now prefer to practice the invention.

25 In accordance with this invention artificial yarn is employed having what I shall call a "super-twist" which I will define below. Some yarns appear on the market already twisted but the super-twist which I give the yarns is higher 30 than that occurring in the usual twisted yarns on the market. In carrying out the first step of the process I may start with a yarn which is either normally twisted or else has no twist at all. After giving the yarn a "super-twist" it is placed on bobbins and in this condition is subjected to setting 35 preferably accomplished by an intensive wetting at high temperature. Thereafter the yarn is carefully dried on the bobbin or spool. After this treatment the yarn is detwisted in the opposite direction and as a rule given more turns in the opposite direction than the yarn had when the detwisting started, so that the prepared yarn shows a twist opposite to the one it originally had. The yarn so prepared has high elasticity 40 and the other characteristics desired, as mentioned above.

In practice twisted yarn, or, as usually the case, especially with cuprammonium yarns, the untwisted yarn is twisted on an appropriate apparatus such as a twisting machine. The amount of twist given to produce the "super-twist" depends on the kind and size of the artificial silk 45 yarn as also on the effect desired, according as more or less curl is sought. For instance, I employ 400—1250 twists per meter for 60—80 denier

size artificial silk to give such silk a "super-twist"; or for size 200—300 denier I employ at least 400—600 twists per meter. I consider it unnecessary and impractical to attempt to state the number of twists for all kinds and sizes of artificial yarns, 5 to give such yarns the super-twist. I have indicated above, as well as in the examples below, super-twists for certain yarns. For other yarns it is an easy matter for anyone skilled in the art to make a simple test on the particular yarn 10 to be treated by twisting it, setting it and untwisting it as herein described, and determining thereby what minimum twist is required to give to the yarn the characteristics herein mentioned as desired. When I refer to "super-twist" given 15 yarn or "super-twisting" yarn, I intend to cover the twists or twisting action necessary for producing such results. In order to obtain very characteristic effects, the number of twists can be considerably increased over the minimum 20 amount. Thereafter the material in the twisted condition is "set" by moistening at high temperature. The twisted yarns are preferably wound on spools of metal or other heat and water-resistant material. The winding on these spools is 25 done preferably in the same operation while the super-twist is being given the yarn.

The important wetting treatment is accomplished at elevated temperatures. For this purpose steaming at atmospheric pressure is especially suitable. This may be done in a steam kettle. In certain cases it is sufficient to place the bobbins or spools in boiling water or in water near the boiling point. In order to facilitate the wetting action, wetting agents can be used. These 30 are either previously introduced in the fiber or are added to the wetting bath. Such agents include sulphurized oils, Nekal, etc. Depending upon the kind of material employed and the wetting method used, the soaking of the material 35 may occur for a shorter or longer period. It is important that after the wetting-out treatment, the yarn on the spool be completely dried.

The untwisting is preferably carried out on a twisting machine or similar apparatus. The degree of untwisting is determined according to the purpose for which the prepared products are to be used. In each case the untwisting is to be carried close to the zero point. For most purposes, it is, however, twisted past the zero point so that 45 the final yarn possesses a given twist but in the opposite direction. In order to save manipulation the reverse twist is carried out only as far as necessary.

The process can be applied to all kinds of arti- 55

ficial silks consisting of untwisted, twisted or spun threads. In addition such threads mixed with other vegetable or animal fibers can be ennobled in this manner. The final product can be used for all purposes for which yarns are employed, such as for cloth, knitting, braiding and embroidery, etc.

Threads treated according to the process of the invention can also be cut to staple fibers and re-spun for which the artificial curled fibers are particularly suited.

The following are given as examples of the process. It is to be understood that the examples are illustrative and are not to be construed in a limiting sense.

#### Examples

1. Copper ammonium yarn of a size of 150 denier with a twist of 200 per meter is super-twisted to 2000 twists per meter. Thereupon the supertwisted yarn, which has been placed on Nickelin bobbins, is steamed at 5 atmospheres pressure for 20 minutes at 158° C. After drying, the yarn is untwisted on the twisting machine, past the zero point and brought to 80 twists per meter in the opposite direction.

2. Viscose yarn of a size of 450 denier with 100 twists per meter is supertwisted to 1200 twists per meter. Then the supertwisted yarn held on spools is steamed at 2 atmospheres pressure for one-half hour at 135° C. The yarn is untwisted after drying past the zero point and brought to 50 twists per meter in the opposite direction.

3. Acetate silk yarn of a size of 120 denier with 150 twists per meter is supertwisted to 2000 twists per meter. The yarn, which is wound on the spools, is now suspended in boiling water and left for one hour in this boiling bath. After careful drying the untwisting of the yarn takes place as mentioned in the previous examples to a final twist of 100 per meter in the opposite direction.

4. Untwisted copper ammonium yarn of a size of 120 denier is given 2500 twists per meter. Then the yarn spools are steamed for 40 minutes at 4 atmospheres pressure at 152° C. After drying the yarn is untwisted to the zero point and in this condition is cut into staple fibers on a suitable cutting machine.

5. Acetate silk yarn of a size of 120 denier with 150 twists per meter, is supertwisted to 2000 twists per meter, then the supertwisted yarn held on spools is impregnated with a wetting agent consisting of Turkey red oil. Thereafter the yarn still wound up on the spools is suspended in boiling water and left for 50 minutes in this boiling bath. After careful drying the untwisting of the yarn takes place as mentioned in the previous examples to a final twist of 100 per meter in the opposite direction.

In the examples given above, the references to "atmospheres pressure" means super-pressure; for instance, the reference to "5 atmospheres" corresponds to 6 atmosphères absolute. Further with respect to the various examples of the invention described above, it is to be understood that the temperature may vary approximately between 100° C. and 160° C. depending upon the atmospheric pressure used while steaming.

70 The yarns prepared according to the invention and particularly as given in the examples above, have a lasting curliness which increases in accordance with the degree of twisting, the increased curliness being desirable for decorative purposes. The elasticity of the yarn is consider-

ably increased and the relative heat-conducting capacity is reduced. By the invention, an effect of increased softness and wooliness is obtained, and also increased heat-insulation, in a woven or knitted fabric produced from such yarn. In general a product is produced of a wool-like character distinguishing itself from real wool by a certain special luster.

Thus while I have described my improvements in detail and with respect to certain preferred forms, I do not desire to be limited to such details or forms since, as will be noticed by those skilled in the art, after understanding my invention many changes and modifications may be made and the invention embodied in widely different forms without departing from the spirit and scope thereof in its broader aspects, and I desire to cover all modifications, forms and improvements coming within the scope of any one or more of the appended claims.

The expression "setting" as used in the appendant claims signifies a moistening of the yarn at an elevated temperature or equivalent treatment thereof and is distinct from the well-known process of drying.

Having thus described my invention, what I claim as new and desire to secure by Letters Patent is:

1. A process for producing a new artificial fibrous material which comprises supertwisting 20 an artificial silk yarn, setting the twist therein and thereafter untwisting the yarn.

2. A process for producing a new artificial fibrous material which comprises setting an artificial silk yarn having a super-twist and thereafter 35 untwisting the yarn.

3. A process for producing a new artificial silk material which comprises supertwisting an artificial silk yarn, wetting this yarn at an elevated temperature, drying the yarn and thereafter 40 twisting it in the opposite direction.

4. A process for producing a new artificial silk fibrous material which comprises twisting artificial silk yarn until it has a super-twist, placing the yarn so twisted on bobbins, moistening it at 45 a high temperature thereon, drying the yarn thereon and afterwards untwisting the yarn whereby a soft woolly material is produced.

5. A process for producing a new artificial silk material, which comprises supertwisting an artificial silk yarn, placing the supertwisted yarn on a spool, immersing the spooled yarn in a moist atmosphere of about 100° C. or more and twisting the yarn in the opposite direction to untwist it.

6. A process according to claim 3 in which the wetting occurs in water at a temperature near the boiling point or above.

7. A process for producing a new artificial silk material which comprises supertwisting an artificial silk yarn, treating the yarn with a wetting agent, setting the twist therein by moistening the yarn at high temperature, drying the yarn and untwisting it.

8. A process according to claim 3 in which the wetting and drying of the yarn is effected on bobbins.

9. A process according to claim 1 in which the artificial threads are untwisted past the zero point and are then given a twist in the opposite 70 direction.

10. A process according to claim 3 in which the artificial threads are untwisted past the zero point and are then given a twist in the opposite direction.

11. A process according to claim 1 in which the treated threads are finally cut into short staple fibers.

12. Artificial fibers characterized by the fact that they possess a lasting curliness, high luster and great softness, said fibers being readily elongatable when subjected to a stretching force and being sufficiently elastic to return to or nearly to their original position upon discontinuance of said stretching force.

13. A woolly material composed of artificial silk alone or admixed with other fibers possessing a lasting curliness, high luster and great softness, such fibers being readily elongatable when subjected to a stretching force and being sufficiently elastic to return to or nearly to their original position upon discontinuance of said stretching force.

RUDOLPH H. KAGL. 10